

Aug. 28, 1928.

1,682,687

F. W. SAMPSON

# CONCRETE BLOCK OR SLAB AND METHOD OF MAKING THE SAME

Filed July 28, 1926

Fig. 1.



Fig. 2.



Inventor

FRANK W. SAMPSON

३४

Ch. Parker

Attorneys

## UNITED STATES PATENT OFFICE.

FRANK W. SAMPSON, OF ATLANTA, GEORGIA.

## CONCRETE BLOCK OR SLAB AND METHOD OF MAKING THE SAME.

Application filed July 28, 1926. Serial No. 125,567.

This invention relates to concrete blocks or slabs and methods of making the same, and particularly to concrete roads and methods of laying the same.

5 It has been the common practice to construct concrete roads of a mixture consisting of coarse rock aggregates and mortar which is poured over the sub-grading and planed or smoothed to the desired surface contour. In 10 using such a mixture, a certain proportion of mortar must be employed to fill the voids between the rock aggregates, and it is the common practice to use an excess of mortar in order that the mixture may be brought to 15 an easily workable form. The durable coarse aggregates of the concrete mixture enveloped in the surface consequently are held apart, and the disturbances of the concrete mixture as it is dropped from the mixing machine to the roadway sub-grade, as 20 well as the further disturbances when the concrete is spread within the form, causes the various pieces of the aggregates to be displaced from their relative position in 25 the mass thus forming rock clusters and consequent mortar pockets in the finished pavement surface. It is well known that the cement and sand mortars of all concrete pavements possess less resistance against destruction under surface wear and impact than the coarse aggregates of granite, trap rock, limestone and other coarse pieces of stone of natural structure, while selected gradings of 30 more durable stone such as those mentioned 35 possess higher and more uniform wear resisting qualities than gravel conglomerate.

It is well known by engineers and road builders that the impact of heavy loads is the quickest and surest destroyer of roads, 40 and consequently engineers are requiring that the surfaces of concrete roads be planed to a substantially perfect contour and grade line in order that the road surfaces may be protected as far as possible against the 45 damaging impact that starts immediately at the point of any surface imperfection. In the concrete pavements built by ordinary methods, as referred to above, the perfectly planed surface affords only temporary protection against destruction by impact, as the 50 tractive thrusts of highway vehicles grind dust and grit against the pavement surface, thus causing continual frictional wear.

This frictional wear eventually disintegrates the finish coat of surplus mortar on the pavement until the coarse aggregate of natural durable stone is reached. Since the stone is more resistant to abrasion than the mortar the rate of wear is very materially reduced 55 in areas where the stones happen to be present at the surface of the road in close proximity to each other, while abrasive wear continues at a relatively rapid rate over areas in the surface where mortar pockets exist or where the stone may be widely separated 60 by the mortar, or where the stone may be sunk below the uniform surface elevation 65 in the surplus mortar. At this point in the life of the concrete road of ordinary construction, the variable rate of wear will soon 70 create unevenness in the pavement surface which will greatly increase the impact forces to which the surface of the road is subjected and hence hastens the destruction of the 75 road.

It also has been proposed to construct concrete roads by laying a sub-base of a mixture containing a lean mortar mixture and rock aggregates of a low grade, and permitting the sub-base to set, after which the surface course is laid and planed. The use of 80 lean mortar mixture and low grade aggregates in the sub-base permits the road more economically to be built, but it has been found that a very imperfect bond is provided between the sub-base and surface course which causes them to separate. It is necessary to permit the sub-base to completely set before laying the top course inasmuch as it is impossible to transport the 85 materials for the top course before the sub-base has set.

It also has been proposed to construct concrete roads with ordinary mixtures containing an excess amount of mortar by pouring the concrete in position and then subjecting it to vibration to cause a wedging action to take place in the aggregates. In the method referred to, and which has been commonly practiced, a layer of concrete mixture containing a surplus of mortar is poured over the sub-grade. A layer of clean high grade aggregates is then spread over the concrete mixture after which the road is subjected to vibration to tamp down the surface aggregates. It has been found in actual prac- 95 100 105

tice that the tamping to which the road is subjected causes some of the higher grade surface aggregates to be driven downwardly a material distance below the road surface, 5 while some of the lower grade base aggregates are caused to rise to the surface. Obviously such lower grade aggregates do not possess the desired resistance to wear, and hence the surface of the road is subjected to 10 the destructive actions of impact and abrasion to a greater extend than if the higher grade rock aggregates only were retained at the surface.

An important object of the present invention 15 is to provide a road including a sub-base and surface course employing low grade and high grade aggregates respectively, and wherein the higher grade aggregates are definitely maintained at the surface of the road to present a durable wearing surface.

A further object is to provide a concrete road which economically may be constructed due to the use of relatively low grade aggregates in the sub-base, and wherein a perfect bond is effected between the sub-base 25 and surface course.

A further object is to provide a road of the character above mentioned wherein a relatively high percentage of the road surface 30 is made up of stone aggregates, as distinguished from the usual concrete road surface which is composed largely of surplus mortar, whereby greater resistance to impact and abrasion is obtained.

35 A further object is to provide a method of constructing concrete roads wherein greatly increased beam strength and improved surface wearing qualities are obtained, thus materially increasing the life of the road by minimizing cracking of the road and destruction of the surface.

A further object is to provide a method 40 of constructing concrete roads wherein a distinct deficiency of mortar mixture is employed as distinguished from the usual practice of employing an excess of the mortar mixture to obtain a more uniform distribution of aggregates throughout the mixture, thus preventing the formation of mortar 45 pockets.

A further object is to provide a method of the character outlined wherein a cement containing sub-base is laid over the sub-grade and is subjected to a vibrating action to 50 wedge the aggregates together and to pour a surface course of mortar and rock aggregates over the sub-base before the latter has set, and to subject the surface course to a 55 vibrating action to cause a wedging action of the rock aggregates therein.

A further object is to provide a method 60 of the character just mentioned wherein the aggregates employed in the surface course are preferably of the flat elongated type 65 whereby an increased lateral wedging takes

place under the influence of the vibration to increase the beam strength of the road.

A further object is to provide a method of coloring the road to a substantial depth below its surface without disturbing the surface, whereby the road glare usually present on concrete roads is eliminated. 70

In the practice of the method, the road is sub-graded in the usual manner and the road width is defined by mold boards or 75 suitable preconstructed curbing, as desired. A mass is then mixed containing relatively low grade aggregates and a relatively lean mortar mixture, and the proportion of the mortar mixture used is somewhat less than 80 that required to fill the normal voids in the loose aggregates. It is also preferred to use a mortar mixture of the stiffest workable plasticity. After the proper preparation and mixing, the material is deposited upon the 85 prepared sub-grade and compacted to the physical limit of vertical and lateral wedging of the stone aggregates by means of vibration. Any suitable means of vibration 90 may be employed, such as the vibrating machines now in use, and the vibrating action need not be described in detail. It should be borne in mind, however, that the vibrating action to which the surface of the sub-base 95 is subjected takes place together with considerable pressure. The portion of the vibrating apparatus which directly contacts with the sub-base obviously defines the shape 100 of the surface thereof.

Immediately after the sub-base is laid, the 105 surface course is "tumbled" into position. This "tumbling" action consists merely in dumping the material for the coat and pulling or pushing it by rakes or the like to 110 spread it evenly over the sub-base to the proper thickness. The mixture for the surface course consists of a relatively rich mortar mixture and high grade aggregates such as granite, trap rock or the like. The 115 proportion of the mortar mixture employed is less than that required to fill the voids in the loose aggregates. This deficiency in mortar is important in the practice of the invention as will become apparent. In selecting the aggregates to be employed, it is preferred that relatively flat elongated stones be employed in order that increased lateral wedging may be obtained. After the surface 120 course is laid in the manner described, it is subjected to vibration and pressure. The subjection of the sub-base and surface courses to vibration and pressure causes the aggregates to be driven into close contact with each other whereby they are wedged together. This wedging action materially 125 reduces the natural voids whereby the mortar in the mixtures, which was originally deficient in proportion is sufficient to fill the reduced voids and a compact mass results in which there is an even distribution 130

of aggregates and wherein the individual stones are closely compacted, being separated by relatively thin veins of mortar. It will be apparent that the placing of the surface course loosely upon the sub-base causes the aggregates of the surface course to assume different relative positions, but when the surface course is subjected to vibration and pressure, the aggregates tend to flatten out horizontally and overlap each other whereby great beam strength is provided.

The deficiency in the mortar prevents it from falling away from the aggregates to form surface pools on the sub-base as well as the surface course, and very little free moisture is present. It has been found therefore that a perfect bond may be obtained between the sub-base and surface course whereby they are effectually prevented from separating. In the impacting action, use is made of the fact that the semi-plastic mortar which coats the stones acts as a lubricant thereby permitting the stones to slide into the closest possible interlocking co-relation under the process of compacting, and thus the aggregates, as loosely measured before mixing, after being lubricated and tightly wedged together will have their physical volume reduced materially in their final position of rest in the concrete mass. This reduction in volume reduces the voids between the stones, thus maintaining the aggregates in close proximity to each other.

It has been found that the flattening out of the aggregates in the surface course, and the use of a deficiency in mortar, permits a completed road to be formed wherein the surface is made up of as high as approximately 90 per cent stone. In practice I prefer to employ stone having a relatively deep color in order that the surface glare may be materially reduced.

As previously stated, the surface course is placed over the sub-base immediately after the latter has been properly subjected to vibration and pressure. The preparation of the concrete mixture of the base in the manner above described, and the compacting of the base to the limits of vertical and lateral wedging of the stone aggregates quickly renders the base fully and uniformly stable and rigid while the cement in the base is fresh and unset. It has been found that the base, constructed as described, is highly stable, and the materials for the surface course may be transported thereover without loosening any of the base aggregates or materially disturbing the surface thereof in any manner. The stability of the base is such that the vibrating action to which the surface course is subjected will not cause the base aggregates to rise to the top of the surface course, and the higher grade aggregates of the surface course will be prevented from being driven downwardly into the base.

The compacting of the base and the great stability thereof forms a firm support for the surface course during the vibrating action to which the latter is subjected. The base acts, in effect, as a nether stone and materially assists in effecting the lateral wedging of the surface aggregates. As previously stated, relatively flat elongated stones are employed as the aggregates for the surface course, and the latter is formed relatively thin, the depth of the surface course usually being from one and one-half to two times the average thickness of the stones employed as the aggregates. Thus the aggregates more readily are caused to assume substantially horizontal positions by the vibration and pressure to which they are subjected, and the lateral wedging of the aggregates is materially increased.

It will be obvious that only a small amount of mortar can be present on the top of the surface course after the completion of the process above described. The finished road surface is then made by brushing over the top of the surface course before the mortar therein has set. In practice, it is preferred to permit the semi-completed road to remain approximately one hour after the completion of the vibrating action before the surface thereof is brushed. In the brushing operation, I prefer to place a small amount of sawdust, sand, or other absorbing medium on the surface coat, and the brushing action carries the absorbing medium over the top of the surface coat and takes up the excess moisture and the relatively small amount of surface cement present. The surface thus presented has been found to be made up of as high as 90 per cent stone, the remaining surface being made up by the thin veins of mortar between the aggregates. The durable stone employed in the surface course provides a true surface and the stones are held rigidly in their relative positions by the integral character of the road whereby it will be apparent that the road is adapted to be subjected to considerable impact and surface abrasion without injury to the road.

I have found that the mortar adjacent the surface of the road constructed in accordance with the present invention readily may be colored to a substantial depth without destroying the smooth continuity of the surface, to minimize the glare from the lighter portions of the road. Mineral mortar coloring is preferably dissolved in water and swept over the completed road surface before the cement therein has attained its final set, and while the mortar is yet moist from mixing. It has been found that the color will penetrate the moist mortar to a sufficient depth to leave a permanent color. Mineral mortar colorings will all fade, but it has been found that the present method leaves a dull tone of the desired coloring, thus eliminating

sunlight and motor headlight glare from the pavement surface.

In the drawings I have shown several forms of road constructed in accordance with the present invention. In this showing,

5 Figure 1 is a sectional perspective view of a completed road,

10 Figure 2 is an enlarged vertical sectional view of a portion of the road, and,

15 Figure 3 is a similar view of a modified form of road.

Referring to the drawings the numeral 10 designates curbings arranged at the sides of the road. As previously stated these 15 curbings may be dispensed with and ordinary mold boards may be employed for confining the road during its construction. A sub-base 11 is arranged between the curbings, and includes rock aggregates 12, preferably 20 of a low grade regardless of their hardness, and the aggregates are bound together by mortar, as indicated at 13. As previously stated, a deficiency in mortar is employed, but the mortar is sufficient to completely 25 fill the voids after the base is subjected to the vibrating action previously referred to. The base is laid on the usual sub-grading 14, which is crowned in the usual manner and the base also may be crowned as indicated 30 at 15.

After the completion of the sub-base, a surface course 16 may be placed in position. The surface course also is crowned as indicated at 17, and the sides thereof are arranged flush with the inner portions of the curbing as will be apparent. The surface course is made up of preferably flat elongated aggregates 18 bonded by mortar 19. The amount of mortar employed in the sur-

40 face course also is less than the amount necessary to fill the normal voids in the surface aggregates, but is sufficient to fill such voids after they have been reduced by the action of the vibration and pressure to which

45 the surface course is subjected in the manner previously described. As shown in Figures 1 and 2, the relatively flat elongated aggregates 18 are caused to assume substantially horizontal positions under the force of the 50 vibratory impacting, and overlap each other throughout the surface course, thus greatly increasing the beam strength of the road. The top surfaces of the upper aggregates 18 form a large percentage of the actual road 55 surface as indicated at 20.

In Figure 3 of the drawings I have shown a road constructed in the manner illustrated in Figures 1 and 2, except that coloring matter is provided for the surface portions of the cement between the surface aggregates. As previously stated, a solution of a mortar coloring is brushed over the surface of the road and this coloring has been found in actual practice to penetrate to a substantial

depth as indicated at 21. Due to the depth 65 to which it penetrates, the coloring will not wear off and thus the road glare is substantially permanently eliminated.

From the foregoing it will be apparent 70 that the present invention contemplates the provision of a road laid in two courses, to

reduce the cost of construction. The aggregates used in the base are of a relatively low grade, while a relatively lean cement mixture preferably is employed. The vi-

bratory action to which the sub-base is sub- 75 jected causes the sub-base to possess a high degree of stability while still fresh whereby the surface course may be laid immediately

after the completion of the base, and the two 80 courses are caused to bond perfectly and will not separate. The use of a deficient amount

of mortar causes the stones to remain in intimate contact with each other, being sep- 85 arated only by relatively thin veins of mor-

tar. The provision of a road surface made up to a great extent of closely placed stones 90 greatly increases the wearing qualities of the road whereby the latter will not be so highly

subject to the destructive action of impact 95 and abrasion. In this connection attention is invited to the fact that it is the customary

practice to employ some means for preventing the escape of the original moisture from 100 the mortar to permit the latter to properly

cure. In connection with the present meth- 105 od, it should be noted that inasmuch as the

surface of the road is made up principally 110 of rock, the rapid evaporation of the origi-

nal moisture from the mortar is prevented 115 and consequently no outside means is neces-

sary to assist in properly curing the road.

The placing of the coloring matter as shown in Figure 3, together with the use of 115 colored stones provides a road which some-what resembles a black pavement in physical appearance, thus materially reducing road glare.

While I have described the method as 120 being particularly applicable to the building of roads, it will be apparent that slabs or blocks of any desired size may be constructed in accordance with the invention for use in other ways, as in building constructions and the like.

It is to be understood that the structure of the road and the methods outlined are 125 to be taken as preferred examples of the same and that various changes may be made therein without departing from the spirit of the invention or the scope of the subjoined claims.

I claim:

1. The method of making concrete structures which consists in placing a base containing aggregates and an insufficient quantity of mortar to fill the normal voids of the aggregates, vibrating the aggregates of 130

the base whereby the mortar content thereof will be sufficient to fill the voids, placing a surface course containing mortar and aggregates on the base before the latter has set, 5 and vibrating the aggregates of the surface course.

2. The method of making concrete structures which consists in placing a base containing aggregates and an insufficient quantity of mortar to fill the normal voids of 10 the aggregates, subjecting the base to vibration and pressure to reduce the voids substantially to the volume of the mortar, placing on said base before it has set a relatively thin surface course containing mortar and relatively flat elongated aggregates, 15

and subjecting the surface course to vibration and pressure.

3. A concrete construction having an outer portion formed of a relatively large percentage of relatively flat elongated coarse aggregates and a relatively small percentage of mortar, said aggregates lying in close relationship to each other throughout the mass of said outer portion and substantially parallel to each other and to the surface of said outer portion and overlapping each other, the surface of said outer portion being formed of substantially 90 per cent coarse aggregates. 20 25 30

In testimony whereof I affix my signature.  
FRANK W. SAMPSON.